

Jan. 21, 1941.

R. E. THOMAS

2,229,146

DRAWSHEET

Filed Sept. 6, 1939



*Fig. 1*



*Fig. 2*

*Raymond E. Thomas*

INVENTOR

*Frank C. Thilberg*

BY

ATTORNEY

## UNITED STATES PATENT OFFICE

2,229,146

## DRAWSCHEET

Raymond E. Thomas, Newburgh, N. Y., assignor to  
 E. I. du Pont de Nemours & Company, Wilming-  
 ton, Del., a corporation of Delaware

Application September 6, 1939, Serial No 293,545

1 Claim. (Cl. 154—54.5)

This invention relates to newspaper printing and more particularly to a new and improved coated drawsheet for impression cylinders of rotary printing presses.

5 In the standard newspaper printing press the cylinder which carries the type is called the plate cylinder. The cylinder which presses the sheet being printed against the plate cylinder is called the impression cylinder.

10 Impression cylinders of rotary printing presses are made of hard unyielding materials, such as metal. In the printing of paper sheets, it is necessary to cover the face of the impression cylinder with a resilient cushion such as cork, in order to compensate for any irregularities in the printing elements, to produce an even printing impression over the entire surface being printed.

15 The covering for the impression cylinder must be smooth, resilient, non-penetrable by printing inks, possess a hard non-cracking and non-peeling surface capable of withstanding pressure application of great force by the plate cylinders with millions of repetitions. Therefore, it is necessary to cover the resilient cork cushion with sheet 20 material called a drawsheet having these desirable properties.

25 It has also been the practice in the printing art to employ a press blanket which comprises a thick felted sheet which has previously been coated with a suitable coating for covering for the impression cylinder, instead of the cork sheet which is covered with the drawsheet. The coated felt blankets are several times more expensive than the cork sheet covered with a drawsheet since the latter may be replaced several 30 times for the cost of a single press blanket.

35 At present it is common to employ woven cotton fabrics as a base for drawsheets. Such cotton fabrics are made from threads being composed of a number of small cotton fibres twisted together to form a single thread. The short fibres, when twisted into a single filament, have many short protruding fibres commonly referred to as lint. In addition to the lint, due to the 40 fact that the cotton fibres are relatively short, the individual threads are not smooth and have a somewhat irregular surface. In weaving, the rough surface of the individual threads causes imperfections in the woven fabric, referred to 45 as slugs and misweaves. These imperfections in the weaving are accentuated in the surface coating and result in a somewhat irregular surface. The drawsheets constructed on a cotton fabric base are therefore undesirable for these reasons.

50 Throughout the specification and claim the term "drawsheet" is used to mean a coated sheet material which is drawn over a resilient sheet previously attached to a rotary impression cylinder used in the printing industry.

55 The object of this invention is to produce a

drawsheet, the outer surface of which is relatively hard but flexible, and non-penetrable by inks or moisture, cleansing solvents such as hydrocarbons, carbon tetrachloride, etc., which are used in the printing art.

60 A further object is to produce a drawsheet the base of which is exceptionally smooth, strong, and sufficiently firm in texture to prevent stretching, but resilient and having the property to return to its normal smooth surface, that is, the position it occupies before being struck by the plate cylinder carrying the type.

A still further object is to provide a drawsheet with improved anchorage of the coating to a new fabric base in which case the said coating is exceptionally smooth, dry, flexible, non-tacky, and 10 resistant to cracking and peeling when subjected to repeated pressure of great force.

The objectives of this invention are accomplished by employing as a base material a fabric 20 the individual threads of which are composed of a great multiplicity of small continuous synthetic filaments twisted together and woven into a textile fabric, and coating the fabric with a plurality of different cellulose derivative coating compositions. Other objects will appear hereinafter.

25 These objects are accomplished by preparing a drawsheet with a special type of fabric which has no slugs or misweaves and which is resilient and elastic. The base fabric is coated with a 30 plurality of compositions which make the finished product smooth and strong and also enhances the strength of the original fabric.

35 A suitable fabric for the present invention is strong rayon, by which I mean a rayon prepared from a regenerated cellulose yarn or cellulosic yarn wherein not more than one hydroxyl group of each C<sub>6</sub> group is substituted, said yarn having a strength of at least 2.5 grams per denier. Usually the strength of the fabric used in practice is about 3 grams per denier which is nearly 40 twice the strength of ordinary rayon.

45 Suitable fabrics prepared from the above described yarn will probably be apparent to those skilled in the art. However, it has been found that fabrics having a construction of 80 x 64, 140 denier, 60 filament, regenerated cellulose are suitable provided the yarn has a strength of over 2.5 grams per denier. Another construction which has been found suitable is 120 x 88 with 100 denier, 100 filament, regenerated cellulose yarn. In these designations the first number refers to the threads per inch in the warp, while the second figures relate to the filling threads per inch. It is also desirable to select fabrics which have 50 a filament size of not more than 2.5 denier.

55 It has been found that a synthetic fabric having a thread count of 85 in the warp direction and 68 in the filler, weighing 3.4 ounces per square 60

yard is very satisfactory for the purpose indicated.

The above described fabric, hereinafter referred to as synthetic fabric, is provided with non-cracking, non-peeling, ink resistant coating, comprising a cellulose derivative as the film forming component. The first two coats consist of a resin-cellulose nitrate solution. The following is given as an example, with the understanding that variations may be made without departing from the scope of this invention.

In the drawing the Figures 1 and 2 represent a diagrammatic section through the coated fabric. In both figures the base fabric is shown as 1, the base coating comprising cellulose nitrate and resin is indicated by 2; the intermediate coating comprising cellulose nitrate, resin and pigment is indicated by 3; and 4 represents a surface lacquer. In Figure 2 a plasticized coat 20 on the opposite side is shown as 5. This coat may have a slight tack. These coatings will be described in detail hereinafter.

#### FIRST COATING COMPOSITION

25

##### Example A

|                                                                                                                         | Per cent by wt. |
|-------------------------------------------------------------------------------------------------------------------------|-----------------|
| 36 oz. cellulose nitrate solution (24.07% cellulose nitrate dispersed in 1 part ethyl alcohol and 1 part ethyl acetate) | 59.3            |
| 65% solution of urea-formaldehyde resin dispersed in isobutyl alcohol                                                   | 10.9            |
| 60% solution of alkyd resin-castor oil modified dispersed in toluol                                                     | 12.3            |
| Butyl acetate                                                                                                           | 17.5            |

The urea-formaldehyde resin may be prepared in accordance with U. S. application Serial No. 58,000, filed January 7, 1936, by D. E. Edgar, et al.

40 The cellulose nitrate employed in the above coating composition has a nitrogen content of 12.3% to 12.5%. The viscosity characteristic is 90 to 110 seconds as determined by the A. S. T. M. D301-33. The urea-formaldehyde resin solution acts as a penetrating agent which assists the composition to penetrate into the threads of the synthetic fabric. The alkyd resin is a plasticizer for the urea-formaldehyde resin and cellulose nitrate.

50 Another example of the first coating composition is as follows:

#### FIRST COATING COMPOSITION

55

##### Example B

|                                                                                                                         | Per cent |
|-------------------------------------------------------------------------------------------------------------------------|----------|
| 36 oz. cellulose nitrate solution (24.07% cellulose nitrate dispersed in 1 part ethyl alcohol and 1 part ethyl acetate) | 44.4     |
| 60% solution of alkyd resin-castor oil modified dispersed in toluol                                                     | 40.6     |

65 Two coats of either of the above compositions are applied to the synthetic fabric by means of a doctor knife. Approximately two ounces of the first coating composition are deposited per square yard of fabric. After each coat the material passes through a heated drying tunnel to expel the volatile components.

70 After the first coating composition is applied, there is deposited a plurality of coats of a plasticized, pigmented, intermediate coating composition, prepared in the following manner: The dry pigments are ground in "Paraplex RG2" resin in the following preparation:

#### MILL BASE (Pigment—Resin grind)

|                                                                                                               | Per cent |
|---------------------------------------------------------------------------------------------------------------|----------|
| Lithopone                                                                                                     | 36.10    |
| Yellow ochre                                                                                                  | 12.04    |
| Bone black                                                                                                    | 6.26     |
| "Paraplex RG-2" resin (castor oil modified sebacic acid glycerol condensation product) in 60% toluol solution | 45.60    |

10 The above ingredients are ground in a ball mill for approximately eight hours or until each individual pigment particle has been wetted. The intermediate coating composition consists of the following:

|                                                                                              | Per cent by wt. |
|----------------------------------------------------------------------------------------------|-----------------|
| Mill base                                                                                    | 17.3            |
| 24 oz. cellulose nitrate sol. (17.44% solution in 1 part ethyl alcohol—1 part ethyl acetate) | 20              |
| "Paraplex RG2" resin (60% solution in toluol)                                                | 61.0            |

15 The cellulose nitrate in the above formula is the same type as that described above in the first coating composition. The "Paraplex RG-2" resin is an alkyd resin and is available on the open market. The ingredients are thoroughly mixed for approximately 30 minutes to obtain a homogeneous dispersion.

20 Immediately following the application of the two coats of the cellulose nitrate-resin first coating composition, there is applied two coats of the above intermediate coating composition by means of a doctor knife. After the volatile solvents have been expelled by passing through a heated chamber, the thus treated material is passed between smooth embossing or calender rolls to improve the anchorage of the coating 40 to the synthetic fabric, and also to smooth out any unevenness in the coated surface. Following the first embossing, four coats of the intermediate coating composition are applied and the volatile components are expelled between each 45 coat by passing through a heated chamber. The material is again subjected to an embossing operation similar to that mentioned above, after which a plurality of approximately ten coats of the intermediate coating composition is deposited. There is applied approximately 20 ozs. of the intermediate coating composition per square 50 yard. The amount of coating will vary depending upon the thickness of the synthetic fabric before coating. Following the final application of 55 the plasticized, pigmented intermediate coating composition, the coated surface is sprayed with a low concentration surface lacquer containing aluminum particles or flakes. The formula for this surface lacquer is as follows:

#### SURFACE LACQUER

##### Example A

|                                                                                                  | Per cent |
|--------------------------------------------------------------------------------------------------|----------|
| 24 oz. cellulose nitrate sol. (17.44% solution in 1 part ethyl alcohol and 1 part ethyl acetate) | 24.4     |
| Butyl acetate                                                                                    | 29.3     |
| Ethyl acetate                                                                                    | 13.31    |
| Flat aluminum particles or flakes                                                                | 3.69     |

70

75

100.00  
Another example of a surface lacquer which results in a dry matte finish is as follows:

SURFACE LACQUER  
Example B

|                   | Per cent |
|-------------------|----------|
| Cellulose nitrate | 4.05     |
| Ethyl alcohol     | 21.37    |
| Ethyl acetate     | 33.03    |
| Cellulose acetate | 4.56     |
| Acetone           | 6.99     |
| Toluene           | 30.00    |

10 The method of preparation of the above composition is disclosed in U. S. Patent 2,169,200, filed November 6, 1937, by F. G. Uhler, and also in U. S. Patent 2,169,199, filed July 22, 1937 by

15 R. E. Thomas. Approximately two ounces of either of the above surface lacquers are applied per square yard.

20 In the preferred embodiment the weight of the synthetic fabric is 3.4 ounces per square yard, the dry weight of the various coatings is 7.0 ounces per square yard and the thickness of the synthetic fabric plus the coatings is approximately .012".

25 After spraying or coating the material with sufficient surface lacquer to cover the intermediate coating and expelling the volatile solvents, the drawsheet is finished and ready for use, or it may be further treated by applying a non-slipping coating composition to the uncoated side or back of the drawsheet as hereinafter described.

30 In practice an impression cylinder is usually too wide to be covered with a single drawsheet, and two separate drawsheets are stretched over the cork covered impression cylinder, and the edge of one sheet is abutted with the edge of the other sheet in the middle of the cylinder. During the continuous pounding of plate cylinder 40 against the drawsheet stretched tautly over the impression cylinder, there is a tendency for the two drawsheets to slip toward the edges of the impression cylinder and become separated due to the smoothness of the continuous rayon filaments which form the back of the drawsheet. The slipping of the drawsheet more than  $\frac{1}{8}$  of an inch 45 is objectionable since this is usually the distance of the printed material from the edge of the paper being printed.

50 In order to prevent slipping of the drawsheet on the cork covered impression cylinder a suitable coating having non-slipping properties is applied on the back side of the fabric which contacts the cork covered impression cylinder. By 55 the way of illustration and not limitation, the following composition has been found satisfactory to apply on the back side of the drawsheet after the face coating has been completed, to prevent the slipping of the drawsheets on the cork covered impression cylinder:

|                        | Per cent |
|------------------------|----------|
| Polyvinyl acetal resin | 19.3     |
| Castor oil             | 12.8     |
| Toluol                 | 24.3     |
| Ethyl alcohol          | 43.6     |

65 A plurality of coats of the above composition are applied to the back side of drawsheet. Approximately four ounces of the above composition are

deposited per yard of material 40" wide, which corresponds to 1.3 ounces of the non-volatile components. Other film forming materials such as other vinyl resins and cellulose derivatives suitably plasticized, which have a slight tack under pressure, may also be satisfactorily used for the non-slipping coating applied on the back side of the rayon fabric.

70 The invention has been described with reference to specific coating compositions which have been given by the way of illustration and not limitation. It is within the purview of this invention to use other types of coating compositions employing other cellulose ester derivatives such as e. g., cellulose acetate, cellulose butyrate, cellulose formate, etc. as well as cellulose ether derivatives, e. g., ethyl cellulose, benzyl cellulose, etc. The drawsheet may be any thickness as long as a substantially plane surface is obtained.

75 An outstanding advantage of a drawsheet produced in accordance with the disclosure of this invention is the extremely firm bond of the coating to the woven base. The resin-cellulose nitrate first coating composition is intended to penetrate into the interstices of the synthetic 25 fabric, and as a result of the penetration of the coating into the fabric, the strength of the bond of the coating to the fabric base is increased.

80 A still further advantage is the high tensile strength of the coated synthetic fabric which allows the coated fabric to be drawn tautly over the cork sheet covering the impression cylinder and while in this taut condition is capable of sustaining pressure application of great force by 35 the printing plates with millions of repetitions without the fibres of the fabric or coating being broken.

85 A still further advantage is the substantially plane surface of the coated drawsheet which results from the use of the synthetic fabric having 40 a substantially plane surface resulting from the absence of lint, misweaves, and slugs.

90 A still further advantage is the improved coating composition for the synthetic fabric. The coating is dry, flexible, non-tacky and substantially 45 resistant to cracking and peeling when subjected to repeated pressure of great force.

95 While the invention has been described in detail with specific examples, such examples are illustrative and are not given as limitations, since other modifications within the spirit and scope of the invention will be apparent to those skilled in the art. Hence, the invention is to be understood as limited only as indicated, in the appended claim, in which the intent is to set forth 55 all the novelty over the prior art.

I claim:

100 A drawsheet comprising a base fabric prepared from threads of regenerated cellulose of uniform denier, on one side of said fabric a base coat 60 comprising a cellulose derivative and an alkyd resin, an intermediate coat comprising a cellulose derivative, alkyd resin and pigment and a surface coat of a dull cellulose derivative composition, on the opposite side of said fabric a plasticized resin coat, said last mentioned coat having 65 a slight tack under pressure.

RAYMOND E. THOMAS.